

1

3,692,522

## ELECTROPHOTOGRAPHIC MATERIAL OF ZINC OXIDE TREATED WITH GUANAZOLE

Robert Joseph Noe, Mortsel, Jozef Frans Willems, Wilrijk, Albert Lucien Poot, Kontich, and Karel Eugène Verhille, Mortsel, Belgium, assignors to Gevaert-Agfa N.V., Mortsel, Belgium

No Drawing. Original application June 6, 1969, Ser. No. 831,253, now Patent No. 3,634,080. Divided and this application July 21, 1971, Ser. No. 164,821

Claims priority, application Great Britain, June 6, 1968, 27,045/68

Int. Cl. G03g 7/00

U.S. Cl. 96—1.8

23 Claims

### ABSTRACT OF THE DISCLOSURE

Electrophotographic recording material containing photoconductive zinc oxide treated with guanazole and processes of electrophotographic recording using such materials. These materials are characterized by low memory effect, improved charging characteristics and are capable of accepting either positive or negative charges to obtain either positive or negative copies.

This invention is a divisional application of the United States Pat. application Ser. No. 831,253 filed June 6, 1969, now U.S. Pat. No. 3,634,080, entitled "Photoconductive Recording Material."

Photoconductive binder type coatings prepared by incorporating a finely divided photoconductor in a binder are well known.

Commonly used are electrophotographic materials containing a photoconductive layer comprising photoconductive zinc oxide dispersed in an insulating binder. Said layer is coated on a sufficiently conductive support, e.g. a clay-coated or glassine type paper base, from a paint-like coating mixture by conventional paper coating techniques. Since the zinc oxide has a brilliant white colour it forms an excellent base for contrasting with the developer materials applied to it. Moreover zinc oxide is relatively less expensive and can be spectrally sensitized by a great variety of dyes. However, as already explained in the United Kingdom patent specification 1,020,504 filed Dec. 29, 1961 by Gevaert Photo-Producten N.V., zinc oxide possesses the less interesting property of having a relatively low dark-resistivity. Hence, in order that the electrical conductivity of a photoconductive recording layer based on photoconductive zinc oxide shall be sufficiently small in the dark for retaining an electrostatic charge during the time needed for exposure and development, it is usual to incorporate in the recording layer some other substance with a higher electrical dark-resistivity.

For that purpose and by the need of a photoconductive recording layer with sufficiently mechanical strength a binding agent is used improving the dark-resistivity of the recording layer.

According to said United Kingdom patent specification, zinc oxide is treated with certain organic phosphorus compounds, preferably organic oxyacids of phosphorus improving the dark-resistivity of the photoconductive zinc oxide grains. By that treatment it is possible to use a larger number of binding agents and even such type of binding agents that have no very low electrical conductivity. As a further result of that treatment the photoconductive recording layer is less sensitive to variations in relative humidity and may contain a much higher amount of photoconductive zinc oxide so that an optimum sensitivity is reached.

Unfortunately the introduction of said organic phosphorus compounds gives rise to a rather large "memory

2

effect" i.e. to a rather large residual conductivity in the time after exposure.

Quantitatively speaking the "memory effect" is expressed here by the ratio of the periods of time ( $t_1$  and  $t_2$  respectively) elapsing before by electrostatic corona charging in the absence of light 90% of the maximal charge level is attained on a photoconductive recording layer that has not been exposed previously (time  $t_1$ ) respectively 90% of the maximal charge level is attained on the same photoconductive recording layer (time  $t_2$ ) that immediately before its charging had received an exposure to active light sufficient to remove a charge that had been applied in a previous step.

The present invention is based on the discovery that the treatment of photoconductive zinc oxide with a guanazole compound (treating agent) corresponding to the following structural formula (including its salt and tautomeric structures):



increases the dark-resistivity of a recording layer containing such zinc oxide and gives rise to a small "memory effect." The said treatment improves the chargeability of a photoconductive recording layer containing photoconductive zinc oxide with a negative corona and moreover besides the possibility of negative corona-charging offers the unexpected possibility of positively corona-charging the recording layer and obtaining thereon positive electrostatic charge images.

Thanks to the property of the recording material according to the present invention of being capable to be charged positively as well as negatively, it is possible with one and the same developer, e.g. an electrophoretic developer with toner particles possessing a particular sign of charge, to reproduce one and the same original at will as a positive or negative copy depending on the sign of the electrostatic charge applied to the recording layer of said recording material.

Thus, it is possible e.g. starting from a microfilm original to prepare positive as well as negative enlarged copies.

The same effects as described above are obtained when the photoconductive zinc oxide is mixed with other photoconductive substances e.g. the photoconductive chalcogenides of cadmium more particularly photoconductive cadmium sulphide, crystalline mixed cadmium sulphide selenide and cadmium selenide. The said chalcogenides may be doped e.g. with zinc in order to increase their photosensitivity.

A small "memory effect" of the recording material is advantageous in cases in which the recording material before its image-wise exposure accidentally or not is overall-exposed to daylight or in which the recording material has to be used in a multicolour reproduction system, wherein the recording layer is several times successively charged and exposed e.g. through halftone selection transparencies of the multicolour original to be reproduced.

According to a practical method of determining the memory-effect the recording material to be tested is fixed onto a rotating disk whereon it is successively carried under a corona charging unit and under a probe or electrode, wherein a charge is induced being directly proportional to the one present on the recording layer (ref. Cassiers, J. Phot. Sci., 10 (1962) 58).

The time ( $t_1$ ) of reaching 90% of the maximal charge level is noted and then the recording material after maximal charging is exposed till complete discharging. Practically immediately thereafter charging is repeated and again the time ( $t_2$ ) is noted for reaching 90% of the sec-

ond maximal charge level which normally is not as high as the one obtained in the first charging step. A usual rotating speed of the disk is 750 r.p.m.

The compound involved can be prepared according to the method described in: J. Prakt. Chemie 88 (1913) p. 310.

In order to achieve an optimum effect, the treating agent is preferably contacted in dissolved form with the photoconductive zinc oxide.

The present invention can be carried out in the manufacture of an electrophotographic recording material, by allowing the zinc oxide to come into contact with the treating agent at any stage of the manufacture. Thus, the contact can take place before or during the preparation of a photoconductive coating composition, comprising photoconductive zinc oxide and a binder material, for forming a photoconductive layer. Alternatively the contact can take place after the formation of the layer e.g. after coating a said compound onto a support.

In order to obtain the desired effects it is not necessary for the treating agent to contact the zinc oxide particles over the whole of their surfaces. Moreover, an electrophotographic recording material according to the invention need not comprise only zinc oxide particles which have been treated in accordance with the invention. The photoconductive layer can incorporate a mixture of treated and untreated zinc oxide grains. Some of the zinc oxide grains can be treated as described in the United Kingdom patent specifications 1,020,504 filed Dec. 29, 1961 and 1,020,505 filed Nov. 8, 1961 both by Gevaert Photo-Producten N.V.

The following methods can successfully be applied for forming a photoconductive layer composition according to the present invention.

(1) The treating agent is added to an aqueous dispersion of the photoconductive zinc oxide. The treated zinc oxide is filtered off or centrifuged, dried and then dispersed in a solution of binding agent. This method is especially suited for compounds that are soluble or dispersible in water.

(2) The photoconductive zinc oxide is dispersed in an organic solvent wherein the treating agent is soluble or dispersible, whereupon the necessary amount of treating agent is added. A binding agent can be applied simultaneously or thereafter.

(3) The photoconductive zinc oxide, a binding agent and a solvent for the latter are dispersed together e.g. by grinding in a ball-mill, according to the particular zinc oxide particle size desired. The treating agent is added before, during or after grinding.

(4) To a paper support a layer is applied from a composition containing the treating agent and optionally a binding agent. Alternatively, the treating agent is incorporated into the paper, e.g. during the manufacture of the paper. On top of this layer (or to the paper as the case may be) a layer is applied containing untreated zinc oxide and a binding agent. During coating of the latter layer and/or during storage of the material some treating agent diffuses from the first layer or the paper backing, to the photoconductive zinc oxide and is absorbed thereon. When this method is used and when a treating agent is employed having a marked antistatic character, the agent can be used in such an amount that a sufficient quantity thereof remains in the paper to render the latter sufficiently conductive for carrying off electrostatic charges during exposure.

(5) To a paper backing is firstly applied a layer of untreated photoconductive zinc oxide, which is dispersed in a binding agent. On top of this layer a layer is applied containing the treating agent and a binding agent if desired. During coating of the second layer and/or during storage of the material, some treating agent diffuses from the second layer to the zinc oxide in the first layer. The composition of the second layer can be selected so

as to impart required surface characteristics to the recording material, e.g. to render the surface suitable for application of the developing processes described and claimed in the United Kingdom patent specifications 1,020,503 and 1,020,505 both filed Nov. 8, 1961 by Gevaert Photo-Producten N.V. It is also possible to use in the second layer a binding agent selected so that the adhesion of a developing powder thereto is either enhanced, thus enabling fixing to be improved, or decreased, thus permitting a better image transfer.

The photoconductive zinc oxide is preferably prepared by the oxidation of zinc vapour, thus is preferably so-called "French-type" photoconductive zinc oxide.

The dark-resistivity of a photoconductive zinc oxide layer can be increased to an optimum value by using increasing quantities of treating agent. If the amount of treating agent, which gives an optimum dark-resistivity, is exceeded, the latter decreases proportionally to the amount of excess treating agent.

It has been established experimentally that an optimum dark-resistivity is obtained by adding to the composition of the photoconductive layer during its manufacture, according to the activity of the selected treating agent (which in that case contains no cations, nor is applied in complexed form) 0.01% to 10% by weight of such agent based on the weight of the photoconductive zinc oxide. Preferably 0.01 to 3% of treating agent is used. The amount of treating agent required when this agent is in salt or complex form is normally higher.

In order to obtain the same effect with corresponding salts or complexed compounds, normally amounts beyond 0.5% by weight in respect of the photoconductive zinc oxide are applied, e.g. between 0.5 and 40%.

It will be understood that if the treating agent is added to a layer or sheet adjacent to the photoconductive layer and allowed to contact the zinc oxide by diffusion, the required proportion of the treating agent in relation to the photoconductive zinc oxide generally is higher than when the treating agent is incorporated into the zinc oxide layer itself.

When a photoconductive layer is formed comprising treated zinc oxide in a binder, the ratio of binding agent to photoconductor influence the quality of the photoconductive layer with respect to the photoconductive properties, mechanical strength and insulating power. It is preferred to employ the binding agent(s) and photoconductor in a weight ratio of from 1:3 to 1:9. If layers are used with a much larger proportion of binding agent, the image sharpness tends to decrease. If layers are used with much lower content of binding agent than the minimum content specified above, the mechanical strength of the coating may be insufficient for many purposes.

The photoconductive recording material according to the present invention can be used in a wide variety of reproduction methods, and enables the production of very contrasty images that can be easily and consistently obtained, even under widely differing circumstances such as strongly varying degrees of air humidity.

In combination with the treating agent used in the present invention binding agents possessing a higher specific dark-resistivity than the treated zinc oxide as well as binding agents possessing a lower specific dark-resistivity can be used. Suitable binding agents are described in the United Kingdom patent specifications 964,878 filed May 3, 1960 and 1,020,054 filed Dec. 6, 1962 both by Gevaert Photo-Producten N.V.

The said treating agent is successfully used in combination with binding agent(s) applied from an organic medium as well as in combination with binding agents applied from an aqueous medium.

Binding agents and mixtures of binding agents suitable to be applied from an aqueous medium are described in our published Dutch patent applications 6608814 and 6608815 both filed June 24, 1966 and 6802733 filed Feb. 27, 1968.

Binding agents and mixtures of binding agents applied from an organic medium are e.g. described in the United Kingdom patent specifications 1,020,503 filed Nov. 8, 1961 and 1,020,504 filed Dec. 29, 1961 both by Gevaert Photo-Producten N.V.

Preferred binding agents contain acidic groups or groups from which an acid can be produced in situ. The content of acidic groups is, however, preferably not so high that the recording layer obtains a water-soluble character.

Very good results are obtained with vinyl copolymers that contain organophilic (hydrophobic) structural units and acidic structural units derived from  $\alpha,\beta$ -ethylenically unsaturated carboxylic acid compounds, e.g. crotonic acid, acrylic acid, maleic acid, itaconic acid and methacrylic acid compounds.

Homopolymers containing acidic structural units may be used in admixture with organophilic polymers. Polymers and copolymers from which acidic groups can be produced in situ contain, e.g. carboxylic anhydride groups e.g. maleic anhydride groups and/or sulphonylchloride groups, which can be hydrolyzed to sulphonic acid groups. The photoconductive zinc oxide is preferably dispersed in an organic medium (aromatic hydrocarbon solvent(s), chlorinated hydrocarbon solvent(s) or lower aliphatic alcholo) by means of an acidic alkyl resin, copoly(ethylene/vinylsulphonyl chloride/vinyl chloride) or formaldehyde acetal of polyvinyl alcohol respectively.

Particularly suitable binding agents and binding agent mixtures for application in recording layers according to the present invention are:

- (1) (a) polyvinyl acetate
- (b) copoly(vinyl chloride/vinyl acetate/maleic anhydride) (85/14/1% by weight)
- (c) copoly(vinyl chloride/vinyl acetate/vinyl alcohol) (91/3/6% by weight)
- (2) (a) copoly(ethylene/vinylsulphonyl chloride/vinyl chloride) (45.2/6.2/48.6% by weight)
- (b) alkyl resin (acid number:12)
- (3) poly(isobutyl methacrylate)
- (4) copoly(methyl methacrylate/isobutyl methacrylate) (20/80 by weight)
- (5) (a) poly(isobutyl methacrylate)
- (b) formaldehyde-acetal of polyvinyl alcohol
- (6) copoly(vinyl acetate/crotonic acid) (94.6/5.4% by weight)
- (7) (a) copoly(vinyl acetate-chrotonic acid) (93.4/6.6% by weight)
- (b) copoly(ethylene/vinylsulphonyl chloride/vinyl chloride) (45.2/6.2/48.6% by weight)
- (8) (a) copoly(vinyl acetate/methyl acrylate/acrylic acid) (67/28/5% by weight)
- (b) copoly(ethylene/vinylsulphonyl chloride/vinyl chloride) (45.2/6.2/48.6% by weight)
- (9) (a) styrolated alkyl resin
- (b) copoly(vinyl chloride/vinyl acetate/acrylic acid) (86.5/13.3/0.2 % by weight)
- (10) copoly(vinyl acetate/methyl acrylate/acrylic acid) (87/12/1% by weight)
- (11) copoly(styrene/methyl acrylate/acrylic acid) (55/44.6/0.4% by weight)

The treating agent applied in the present invention does not exclude the increase of photosensitivity of the recording element, e.g. by spectral sensitization of the photoconductive zinc oxide.

Spectrally sensitizing dyes can be allowed to adsorb to the photoconductive zinc oxide before, during and/or after the dark-resistivity increasing treatment. Spectral sensitizing agents which can be applied are described in the already mentioned United Kingdom Patent specification 1,020,504 and in our published Dutch patent applications 6717400 filed Dec. 20, 1967, 6805983 filed Apr. 26,

1968, 6704706 filed Apr. 3, 1967 and 6704768 filed Apr. 4, 1967. A very suitable technique for applying the spectral sensitizing agents is described in the published Dutch patent application 6704768 which technique can also be applied successfully in respect of the dark-sensitivity increasing compounds used according to the present invention.

The photoconductive recording layers containing a treating agent for photoconductive zinc oxide as described 10 may contain in addition to the photoconductive substance and binder any other type of dark-resistivity or sensitivity increasing compound e.g. the phosphorus compounds and other dark-resistivity increasing compounds described in the Belgian patent specification 612,102 filed Dec. 29, 15 1961 by Gevaert Photo-Producten N.V., and additives known in coating techniques e.g. dispersing agents (see e.g. our published Dutch patent application 6712156 filed Sept. 5, 1967), compounds influencing the gloss and/or the wear resistance of the coating, and compounds that counteract aging and/or oxidation of the layer, or that influence the thermal stability. When selecting any additives, preference is given to those which least reduce the sensitivity and dark-resistivity of the photoconductive layer.

The photoconductive composition treated according to the present invention may be coated on a support according to a known coating technique, e.g. by spraying, whirling, dip-coating, or by a coating technique wherein use is made of a doctor blade. The supports or base materials are chosen in view of the particular charging, exposure, recording and/or transfer technique wherein the recording material is used.

In electrophotographic recording techniques, wherein the photoconductive layer is electrostatically charged, the 35 support has an electric volume resistivity lower than that of the recording layer, preferably at least  $10^2$  as low as that of the photoconductive recording layer. Suitable supports are described, e.g. in the United Kingdom patent specifications 995,491 filed Mar. 16, 1962, 1,020,503 filed 40 Nov. 8, 1961 and 1,020,504 filed Dec. 29, 1961 all by Gevaert Photo-Producten N.V. and in the United States Patent No. 3,008, 825 of Warren G. Van Dorn and Osmar A. Ulbrich, Jr., issued Nov. 14, 1961. Preferably used supports are conductive paper supports, more preferably 45 glassine type paper supports.

The photoconductive layer of an electrophotographic material which is prepared by starting from a coating composition according to the present invention, can be used for recording purposes, in which prior to exposure an electric charge is non-differentially applied according to 50 known methods. However, the material can also be used in recording techniques, in which the exposure step precedes the charging step. For such a technique we may refer to, e.g., the United Kingdom patent specifications 1,033,419 and 1,033,420 both filed Nov. 26, 1962 by Gevaert Photo-Producten N.V.

The charging as already explained can be effected with a negative as well as with a positive corona.

A corona charging system suited for a rapid change 60 from negative to positive corona charging operates with a so-called floating earth having corona wires of opposite charge sign under and in front of the recording layer to be charged.

Well established methods of developing electrostatic images include cascade-, powder cloud-, magnetic brush- and fur brush-development. These methods are based on the application of charged dry toner to the surface bearing the electrostatic image. Other methods are based on the use of liquids, either insulating (electrophoretic development is preferred) or conductive liquids (see e.g. the United States Pat. No. 2,907,674 of Kenneth A. Metcalfe and Robert J. Wright, issued Oct. 6, 1959 and the Belgian patent specifications 610,060 filed Nov. 8, 1961 and 625,335 filed Nov. 27, 1962 both by Gevaert Photo-Producten N.V.). Development of a conductivity image based

on electrolysis is described e.g. by J. A. Amick, RCA Rev., 20, 753 (1959).

The present invention is further illustrated by the following example.

#### EXAMPLE

360 g. of copoly(vinyl acetate/crotonic acid) (95.7/4.3% by weight) were dissolved in a mixture of 21.4 l. of dichloroethane and 1.6 l. of ethanol. To the solution of the binder 12 kg. of photoconductive zinc oxide (French type) of an average particle size of  $0.15\mu$ , and 8 l. of methyl isobutyl ketone were added. The obtained mixture was homogenized in a sand-mill, and to 43.280 kg. of the obtained dispersion were added whilst stirring:

88.8 ml. of a 10% by weight solution of guanazole in 15 dimethylformamide

1665 g. of Hypalon 30 (trade name for a copoly(ethylene/vinylsulphonyl chloride/vinyl chloride) (26.1/6.9/67% by weight) marketed by E. I. du Pont de Nemours & Co. Inc., Wilmington, Del., U.S.A.) dissolved in 20 8.325 l. of sym.-dichloroethane, 162 ml. of a 0.5% solution of



in dimethylformamide

45.5 ml. of a 1% by weight solution of bromophenol blue in methanol.

The obtained dispersion was applied by knife coating to a conductive paper base of 67 g./sq. m. at a rate of 25 g. of solids per sq. m. The obtained layer was dried at 80° C.

The dried recording layer was negatively corona-charged till -600 v. with a double corona, the corona wires in front of the recording layer and those below the support having a potential difference of -5000 v. and +5000 v. respectively in respect of the ground.

The charged recording layer was projection-exposed for 10 sec. by means of an incandescent tungsten filament lamp of 400 watt placed at a distance of 40 cm. through a positive linework transparency and developed by means of an electrophoretic developer as described hereinafter.

A positive 7X enlarged reproduction of the positive transparency was obtained.

The same recording layer was positively corona-charged till +500 v. with the same double corona unit, of which the corona wires in front of the recording layer and those below the support had a potential difference of +5000 v. and -5000 v. respectively in respect of the floating earth.

The positively charged recording layer was exposed in the same optical enlarger as described above but to a negative microfilm images as an original.

By using the developer as described hereinafter a 7X enlarged reproduction having reversed image values in respect of the negative microfilm image was obtained.

The developer was produced by diluting the concentrated developer composition described hereinafter in a volume ratio of 15/1000 by means of Isopar H (trade name for an isoparaffinic hydrocarbon mixture having a boiling range of 177-178° C., sold by Esso Belgium N.V., Antwerp, Belgium):

Carbon black (average particle size: 20 nm.) ---g--- 30  
Zinc monotridecyl phosphate as dispersing agent ---g--- 1.5  
Isopar H (trade name) -----ml--- 750  
Resin solution prepared as described hereinafter ---g--- 150

The resin binder solution was prepared by heating 500 g. of Alkydal L 67 (trade name of Farbenfabriken Bayer A.G., Leverkusen, W. Germany, for a linseed oil-modified

(67% by weight) alkyd resin and 500 ml. of white spirit containing 11% by weight of aromatic compounds at 60° C. till a clear solution was obtained and by subsequent cooling.

5 We claim:

1. A recording process wherein an information-wise pattern of increased conductivity is produced in a photoconductive insulating recording element comprising photoconductive zinc oxide treated with a compound corresponding to the following structural formula and the salt form and tautomeric structures thereof:



15 by steps comprising information-wise exposing said recording element to active electromagnetic radiation.

2. A method for recording and reproducing information comprising the step of forming an information-wise electrostatic charge pattern by electrostatically charging and 25 information-wise exposing to active electromagnetic radiation an electrophotographic recording material containing a photoconductive recording layer comprising photoconductive zinc oxide treated with a compound corresponding to the following structural formula and the salt form and tautomeric structures thereof:



35 3. A method for recording and reproducing information according to claim 2, wherein the electrostatic charge pattern formed on said layer is made visible by development with electrostatically attractable material.

40 4. A method for recording and reproducing information according to claim 2, wherein the recording layer has been applied to a conductive layer or support having a volume resistivity lower than that of the dark-adapted recording layer.

45 5. A method for recording and reproducing information according to claim 4, wherein the support is a paper support.

50 6. A method for recording and reproducing information according to claim 1, wherein the photoconductive zinc oxide is used in admixture with a substance increasing its spectral sensitivity.

55 7. A method for recording and reproducing information according to claim 2, wherein said compound is used in admixture with the photoconductive zinc oxide in an amount of 0.01 to 10% by weight in respect of the photoconductive zinc oxide.

60 8. A method for recording and reproducing information according to claim 1, wherein the photoconductive zinc oxide has been dispersed in a binder medium containing at least one binding agent comprising acidic groups or groups from which an acid can be produced in situ.

65 9. A method for recording and reproducing information according to claim 8, wherein said binding agent is a vinyl copolymer containing hydrophobic structural units and acidic structural units derived from  $\alpha,\beta$ -ethylenically unsaturated carboxylic acid compounds.

70 10. A method for recording and reproducing information according to claim 8, wherein the groups from which an acid can be produced in situ are carboxylic anhydride groups or sulphonyl chloride groups.

11. A method for recording and reproducing information according to claim 2, wherein the photoconductive zinc oxide has been used in admixture with an organic oxyacid of phosphorus increasing the dark-resistivity of the photoconductive zinc oxide.

12. A method for recording and reproducing information according to claim 2, wherein the recording layer is electrostatically negatively charged.

13. A method for recording and reproducing information according to claim 2, wherein the recording layer is electrostatically positively charged.

14. A method for recording and reproducing information according to claim 12, wherein after charging and information-wise exposure the formed electrostatic charge pattern is developed electrophoretically.

15. A method for recording and reproducing information according to claim 13, wherein after charging and information-wise exposure the formed electrostatic charge pattern is developed electrophoretically.

16. A recording material containing photoconductive zinc oxide treated with a compound corresponding to the following structural formula (including its salt and tautomeric structures):



17. In an electrophotographic process for the production of positive or negative reproduction selectively of an original by means of (1) a same photoconductive recording material and developing material having a particular electrical charge polarity and (2) by the choice of the polarity of the electrostatic charge applied to the photoconductive recording element of the photoconductive recording material, the improvement which comprises the use of a photoconductive recording element comprising photoconductive zinc oxide that has been treated with a

5 compound corresponding to the following structural formula (including its salt and tautomeric structures):



10 18. A recording material according to claim 16, wherein the photoconductive zinc oxide has been dispersed in a binder medium in a ratio by weight of from 1:3 to 1:9.

15 19. A recording material according to claim 16, wherein the photoconductive zinc oxide has been dispersed in a binder medium containing at least one binding agent comprising acidic groups or groups from which an acid can be produced in situ.

20 20. A recording material according to claim 19, wherein said binding agent is a vinyl copolymer containing hydrophobic structural units and acidic structural units derived from  $\alpha,\beta$ -ethylenically unsaturated carboxylic acid compounds.

25 21. A recording material according to claim 19, wherein the groups from which an acid can be produced in situ are carboxylic anhydride groups or sulphonyl chloride groups.

25 22. A reproducing material according to claim 16, wherein the photoconductive zinc oxide has been used in admixture with an organic oxyacid of phosphorus.

30 23. A recording material according to claim 16, wherein the photoconductive zinc oxide has been spectrally sensitized.

#### References Cited

##### UNITED STATES PATENTS

2,218,077 10/1940 Zerweck et al. ---- 260—308 C  
3,287,116 11/1966 Hoegl.

35 GEORGE F. LESMES, Primary Examiner

M. B. WITTENBERG, Assistant Examiner

U.S. CL. X.R.

40 96—1 PC; 252—501; 260—308 R

UNITED STATES PATENT OFFICE  
CERTIFICATE OF CORRECTION

Patent No. 3,692,522 Dated September 19, 1972

Inventor(s) Robert Joseph NOE et al

It is certified that error appears in the above-identified patent and that said Letters Patent are hereby corrected as shown below:

Column 9, Claim 16, in the formula, correct to read as follows:



Column 10, Claim 22, line 25, change "reproducing" to -- recording ---.

Signed and sealed this 8th day of May 1973.

(SEAL)

Attest:

EDWARD M.FLETCHER, JR.  
Attesting Officer

ROBERT GOTTSCHALK  
Commissioner of Patents